

May 28, 1940.

J. E. ARBERRY

2,202,682

WRITING SURFACE

Filed March 25, 1939

*Fig. 1.*



*Fig. 2.*



INVENTOR  
JAMES E. ARBERRY  
BY *Olen E. Bee*  
ATTORNEY

## UNITED STATES PATENT OFFICE

2,202,682

## WRITING SURFACE

James E. Arberry, Pittsburgh, Pa., assignor to  
 Pittsburgh Plate Glass Company, Allegheny  
 County, Pa., a corporation of Pennsylvania

Application March 25, 1939, Serial No. 264,159

5 Claims. (Cl. 35—66)

The present invention relates to media for reception of chalk markings and designs and it has particular relation to the provision of boards or tablets suitable for use as blackboards and 5 slates in schools, or for similar purposes.

One object of the invention is to provide a writing board or tablet which is light of weight, durable, and resistant to breakage.

A second object is to provide a board or tablet 10 of the foregoing type, the surface of which is capable of receiving clear and distinct markings from crayons, which markings can be easily and completely erased from the surface by means of felt, or similar erasers, without leaving objectional smudge.

A third object of the invention is to provide a board or tablet for receiving writing from crayons, which board presents a smooth, satiny surface of a desired color.

20 These and other objects of the invention will be apparent from consideration of the following specification and the appended claims.

For the production of school or similar blackboards and slates capable of receiving markings 25 by chalk, crayons, slate pencils and the like, a large number of materials have been suggested. However, none of these is completely satisfactory from all view-points. Among the requisites of a good blackboard or slate are:

30 1. The ability readily to receive or take chalk marks. This has heretofore entailed the presence of a certain amount of gritty or abrasive material in the surface of the board.

2. Chalk marks must be easily erased with a 35 felt, or cloth, or other body of similar texture, without leaving permanent streaks ingrained in the surface and without leaving excessive and sharply defined smudges after the erasure.

3. The surface must be permanent and must 40 not tend to assume an objectionable polish which will not take chalk or crayon marks and which will be characterized by excessive reflections.

4. It is desirable that the board be of a pleasing 45 color that harmonizes with the general motive of the room in which it is employed. In recent years the tendency has been to employ lighter colors in school room decorations, in order to impart an atmosphere of light and cheerfulness to the room. Accordingly there has been a growing need for a board of corresponding color.

Probably slabs of natural slate have, heretofore, more satisfactorily met the most essential requirements of a blackboard or school slate than any other material.

46 However, even it is objectional in certain re-

spects. For example, it is heavy, cumbersome, expensive and easily broken. Moreover, no choice of color is available. These slates are uniformly dark and therefore cannot be employed to increase the brilliancy of motive in a room. 5 Moreover, it will be obvious that the black surface is not suitable for use with many colors of crayons, or pencils.

The present invention involves the discovery 10 that the smooth, satiny apparently gritless surfaces of oxidized or anodized plates or sheets of aluminum possesses the essential requisites of a blackboard or slate to a remarkable degree and in spite of the satiny finish will take chalk or crayon marks with ease. Moreover, the marks 15 can readily be expunged or erased without leaving objectionable streaks or smudges. Furthermore, the surface film is found to be exceedingly hard and resistant to abrasion so that objectional polishing does not occur even after prolonged 20 use.

For a better understanding of the invention reference may now be had to the accompanying drawing in which

Figure 1 is an elevational view of a blackboard 25 embodying the invention.

Figure 2 is a fragmentary cross-sectional view of a portion of the board showing the different layers of materials embodied therein.

In the drawing like numerals refer to like parts. 30

The writing surface such as a blackboard 10 cemented or mounted upon a wall 11 includes a plate or plaque 12 of aluminum of any desired thickness, grade and finish. This plate may comprise a simple plate of aluminum or a plate of 35 steel or other material surfaced with aluminum by electrolysis or other method. The aluminum surface is provided with a smooth, satiny uniform aluminum oxide film 13 which may be formed thereupon by any conventional process 40 of forming oxide films. The common method is the so-called anode processes in which the aluminum body is made the electrolytic anode in a bath of acid, such as chromic acid. The conventional "Alumilite" process is particularly sat- 45 isfactory for the purpose. This process is well understood by those skilled in the art and need not be described in detail. A frame for the board is indicated at 14.

As previously indicated the oxide films upon 50 the aluminum plates are smooth and satiny in feeling and appearance, which is quite different from slates and other common applicable materials, which in general must have a certain amount of grit or grain in order to make them 55

receptive to chalk or crayon markings. The marks may be expunged or erased with an ordinary felt, cloth, or other eraser without any objectional streaking or smudging. Although the 5 film is comparatively thin it is none the less of great hardness and durability to abrasion. Therefore, it is capable of withstanding long and severe usage without failure. In event of ultimate failure it is an easy matter to remove the 10 plates or plaques from the wall and reanodize them in order to provide a fresh working surface.

Oxide coatings upon slabs or plates of relatively pure aluminum are inherently of a silvery appearance and blend and harmonize most excellently with lighter shades of paint or varnish in 15 a room. With such boards it is desirable to employ a black or colored crayon or chalk for marking purposes. By alloying the aluminum with silicon or other metal it is possible to form an 20 oxide film upon the plate of darker hue which will be satisfactory for use with white chalks or crayons.

These oxide films upon aluminum plates are characterized by the ability to take dyes and pigments in order to provide practically any desired 25 color for the film. It thus becomes possible by employing any of the conventional processes of dyeing to provide a board of any color. It is also possible to form designs in the aluminum film 30 merely by applying a dye or pigment by printing or other processes thereof. Permanent guide lines constitute examples of such designs and are indicated at 15 in the drawings. It is also possible to dye parts or all of the board to one shade 35 and to imprint designs of another color thereupon.

It is possible to employ the oxidized plates or sheets not only as school slates or blackboards,

but as score cards for card and similar games, or for practically any purpose where it is desirable to provide a tablet or plaque from which crayon or chalk marks can easily be expunged.

The form of the invention herein shown and 5 described is merely illustrative; many modifications may be made therein without departure from the spirit or scope thereof.

What I claim is:

1. A writing surface for receiving chalk markings comprising a plate of aluminum having a smooth, satiny surface comprising an adherent film of aluminum oxide, said surface being capable of receiving chalk marks, the marks being readily erasable therefrom. 10

2. A wall blackboard for receiving chalk markings comprising a plate of aluminum having a writing surface comprising an adherent anodic film of aluminum oxide, said film being capable of readily receiving crayon marks, such marks 20 being easily erased therefrom by means of a felt or similar eraser.

3. A writing surface as defined in claim 1 in which the aluminum oxide film is impregnated with a dye of desired color. 25

4. A writing surface as defined in claim 1 in which the aluminum oxide film is impregnated with a dye to provide contrasting designs upon the surface thereof.

5. A blackboard for receiving crayon markings 30 comprising a plate of aluminum having a frame and being secured upon a building wall and having a writing surface comprising an adherent anodic film of aluminum oxide, said film being capable of readily receiving crayon marks, such 35 marks being easily erased by means of felt or similar erasers.

JAMES E. ARBERRY.